

## UNITED STATES PATENT OFFICE

HAROLD J. ROSE, OF PENN TOWNSHIP, ALLEGHENY COUNTY, PENNSYLVANIA, AND  
WILLIAM H. HILL, OF NEW YORK, N. Y., ASSIGNORS TO THE KOPPERS COMPANY,  
OF DELAWARE, A CORPORATION OF DELAWARE

## IMPREGNATED PRODUCT AND PROCESS OF MANUFACTURE

No Drawing.

Application filed May 18, 1929. Serial No. 362,880.

This invention relates to improvements in impregnated products and a process of manufacturing the same and more particularly to the impregnation of porous materials with compositions containing coal and/or solutions of coal.

Porous materials such as wood, fabrics made of any kind of fibre, paper, kraft paper, cardboard, felt, prepared porous compositions 10 of various kinds, porous brick or stone, concrete, coke, etc., may be impregnated with coal or coal solutions for the purpose of making them water-proof, resistant to decay or corrosion; for the purpose of strengthening 15 and toughening them; to produce an improved wear surface; and for frictional, adhesive or decorative purposes.

As set forth in our application Serial No. 97,467, filed March 25, 1926, coal may be dissolved in oils, such as coal tar or water-gas tar, and certain distillates therefrom. The coal and oil are brought together and heated 20 at normal or only moderately elevated pressures and moderately elevated temperatures 25 of from about 200° C. to about 400° C. Substantially all of the coal dissolves forming homogeneous solutions which remain stable at temperatures below the point of rapid volatilization, or even below the dissolving 30 temperatures. The coals most easily dissolved in such solvents are generally the coking coals. Substantially all of such coals are soluble, the insoluble portions consisting of the mineral matter or ash and mineral 35 charcoal or "fusain" which may be present in limited amount.

Preferably high boiling coal tar oil or water-gas-tar oil containing resinous material is used as a solvent for coal. Petroleum 40 oils, preferably the products from cracked petroleum oils and especially the higher boiling distillates thereof are also used.

A coal solution suitable for use in the present invention may be prepared by heating about 20 to 25 parts of coal in about 75 to 80 parts of high boiling coke-oven-tar oil, in a closed vessel heated directly to a temperature of about 300° C. Water and undesirable light oils are allowed to escape before the vessel is closed. Large quantities 50

of coal solution may be prepared in advance in which case it may be discharged into moulds and allowed to cool or solidify and stored for later use.

After the resulting product is cooled, it is in a solid or semi-solid state and for impregnation purposes the fluidity thereof may be increased by heating or by the addition of thinning material such as water-gas tar oils or coal tar oils and the like.

Certain thinning materials called introfiers may also be added. Introfiers are substances which promote the penetration of liquids into porous materials or which produce a thinning effect out of proportion to the amount added. Orthochlorphenol and benzyl alcohol, for instance, have this effect and may be added preferably to the extent of about five percent by weight.

Water may also be used as a thinning agent, in which case the coal solution may be in the form of an emulsion.

Coal solution gels prepared in accordance with the disclosure in a copending patent application to William H. Hill, Serial No. 393,115, filed Sept. 15, 1929, now Patent No. 1,875,458, may be used instead of coal solutions as such. One method of preparing such gels or so-called coagulated coal solutions, is as follows: A fairly concentrated coal solution, comprising 30 parts of coal in 70 parts by weight of dehydrated coke oven tar, is crushed as fine as possible and digested with one-quarter of its weight of solvent naphtha for about twenty-four hours. The resulting mass is homogenized in a mixing machine and then run through a colloid mill.

Impregnation with coal solutions of any desired consistency may be carried out at atmosphere pressure, or reduced or elevated pressures, or an alternation of high and low pressures may be used. The material to be impregnated may be heated and/or evacuated before the treatment with coal solution occurs.

The porous material may be impregnated with a coal solution or with a dissolving oil before impregnation with a coal solution which would otherwise wet the material with greater difficulty.

For certain purposes, a complete penetration of the coal solution into the porous material may not be necessary or may be undesirable. In such cases, the penetration may be restricted to a limited depth from the outer surfaces. Furthermore, the interstices or voids in the material treated may be partially filled with a coal solution composition or may be entirely filled. Again, merely the surfaces of the material surrounding the voids or as in the case of fibrous materials, the individual fibres may be merely coated. In certain cases, the individual fibres themselves, especially those of cellular structure, may be impregnated.

The fibres used in connection with this invention may be vegetable fibres such as cotton or grass, animal fibres such as hair or wool, or mineral fibres such as asbestos or mineral wool. The fibres may be loosely or densely matted or woven into webs or pads or may be in the form of blocks, sheets or laminations.

The material treated, especially when in the form of thin objects, may be saturated with the coal-solution composition by submerging the material in the composition in liquid form. Where restricted penetration is desired, the surfaces of the objects may be coated with the coal solution composition and the coated material run through cold or heated rollers, or the coal solution composition may be applied with the aid of rollers to one or both sides of the article. This treatment is especially adapted to the continuous treatment of lengths of material such as cloth, tape, cord, paper, asbestos products, etc.

Limited penetration may also be obtained by brushing or spraying a coal solution composition on the article to be treated and permitting it to soak in. Coal solution paint compositions may be very satisfactorily used in this way.

For certain purposes, a porous material may be partially or wholly impregnated with a coal solution composition and a layer of a coal solution composition placed over the surface of the impregnated material. The porous material may be used in this case for reinforcement purposes.

After the impregnation of articles with coal solution compositions, a part or all of the solvents may be removed by a proper heat treatment with or without the recovery of the solvents. For instance, it may be found desirable, for ease of application, to impregnate articles with a more dilute coal solution than would be desired in the final product. In such cases, a subsequent removal from the impregnated material of some of the solvent could be resorted to as indicated above, thus leaving a residue of concentrated coal or coal solution in the pores.

Coal may be precipitated from solution by

the addition of volatile organic liquids such as gasoline, naphtha, turpentine, etc. After impregnation, the coal may be precipitated, when desired, in the pores of the material treated by saturating with these organic liquids.

The drying of the impregnated material or the removal of solvents or thinners may be accomplished by use of vacuum, by heating, by treating with steam or other carrying gases, or by any combination of these treatments.

The quality of certain products impregnated with coal solution compositions may be improved by incorporating in the coal solution, in various proportions, finely divided mineral fillers, finely divided coal or coke, or organic materials either soluble, such as resin, or insoluble materials, such as cellulose particles, or wood-flour. Substances such as rubber or latex materials may also be incorporated in the impregnating mixture. It is advantageous to include aging or curing substances such as sulphur or sulphur compounds which will tend to toughen or harden the material during the above mentioned heat treatment or after a lapse of time. Accelerators such as diphenylquanidine or thiocarbanilide may be used if desired. Alternatively, coal solution or the oil used as solvent may be treated with sulphur before using it as an impregnating medium.

Porous compositions containing coal may be impregnated with a solvent for coal or with a coal solution. When using solvent alone, the coal may be made to dissolve therein by further treatment or while in use. Also when a composition is prepared from coal and a solvent therefor and is put to use under favorable conditions, the coal will go into solution.

Porous materials impregnated with coal solution compositions are adapted to be used in many ways. An improved friction tape or shoemaker's thread of tough and enduring quality may be prepared as indicated above.

Cotton tape, for instance, is immersed in a warm solution of coal and the saturated tape squeezed between warm metal rollers. The tape may then be passed through a drying oven at about 100° C. or left in the open for a sufficient length of time to produce a proper surface. Cotton thread may be immersed in a warm solution of coal and the saturated thread drawn through a small orifice to remove excess coal solution.

A very practical application of the present invention consists in treating wood or lumber with a solution of coal in creosoting oil or in oils which contain a large percentage of creosoting oil and/or other materials toxic to fungi and bacteria. This treatment tends to water-proof the wood and preserve it against decay just as in the case of any plain

creosoting oil. However, the presence of coal reduces the solubility of the creosote in water and thus helps to reduce the loss of creosote, due to leaching out by water. As 5 a matter of fact, substantially any coal solution as a normal constituent contains material which inhibits decay, whereas asphalt per se has no such preservative action. Incidentally the cracks in the timber treated 10 become filled with the coal solution and the latter forms an effective sealing means.

In using coal solution compositions as a preservative, they may be employed as sealing compositions for preserving articles by 15 enclosing them in a jacket of porous material such as paper, or cloth made air-tight by impregnating the porous material with a coal solution composition. When sealing food products, a coal solution containing wood tar 20 or wood tar products may be preferred.

Another application of the present invention is in the production of brake bands, 25 brake linings, brake blocks, etc., for automobiles, railway vehicles and other purposes. In preparing such articles, asbestos fabric, formed or matted asbestos fibre, or other porous compositions, may be impregnated as 30 described above. If desired, part or all of the oil content of the brake bands and the like, may be removed by direct heating, steaming, extraction, or treatment with liquids which will render the coal insoluble.

Partial or complete carbonization of the coal may be resorted to by further application of heat.

Mulch paper used for agricultural purposes may be considerably improved by impregnating it with a coal solution composition. 70

Porous materials impregnated with coal solution compositions may be employed also in the manufacture of shingles or other roofing materials, expansion joints, rail fillers, 75 floor cloth, and so forth.

We claim as our invention:

1. A porous material having carbonized coal in its pores, said coal having been previously in dissolved condition. 80

2. A process of preparing an impregnated porous material, which comprises impregnating the porous material with a coal-solution composition containing coal and a solvent therefor, and heating the resulting product to remove solvent and to carbonize the coal. 85

In testimony whereof, I have hereunto subscribed my name this third day of May, 90 1929.

HAROLD J. ROSE.

In testimony whereof, I have hereunto subscribed my name this seventh day of May, 95 1929.

WILLIAM H. HILL.